

## 1

3,672,930

PROCESS OF TRANSFERRING AN ELECTRO-  
STATIC CHARGE PATTERN WITHOUT USING  
EXTERNAL PRESSURE OR ELECTRICAL BIAS  
William Trachtenberg, Rochester, N.Y., assignor to  
Eastman Kodak Company, Rochester, N.Y.  
No Drawing. Filed Apr. 2, 1970, Ser. No. 25,246  
Int. Cl. G03g 13/18

U.S. CL. 117—37 LE

13 Claims

### ABSTRACT OF THE DISCLOSURE

A high resolution process of transferring and developing electrostatic charge patterns is described. An electrostatic charge pattern is formed on an image-bearing member having a very low Sheffield Smoothness value. A receiving element is provided which also has a low Sheffield Smoothness value. The smooth surfaced member is then placed in face-to-face contact with the receiving element in the presence of a thin layer of an electrically insulating isoparaffinic hydrocarbon transfer liquid having a boiling point in the range of 105 to 260° C. During contact, the charge pattern is transferred to the receiving element in the absence of external pressure or electrical bias potential. The transferred image is then developed to form a high resolution visible image.

This invention relates to electrostatic imaging procedures and more particularly to procedures for transferring and developing electrostatic charge patterns.

In the art of electrography, a sensitive element is used which is typically in the form of an electrophotographic element. Suitable elements comprise a conductive support having thereon a layer of a photoconductive composition generally comprising a resinous binder and a photoconductor which may be organic or inorganic and which will accept and retain an electrostatic charge when in darkness. A suitable electrostatic charge is placed on the sensitive element by, for example, subjecting the element to a corona discharge. After charging, such an element is given an imagewise exposure by any suitable means. The exposure results in a variation in the charge on the element in accordance with the relative energy received by the element during exposure. This charge pattern is usually referred to as an electrostatic charge pattern. The charge pattern can now be rendered visible by the application of a suitable developer containing electrostatically attractive marking particles which are drawn to the element in accordance with the charge pattern thereon. The visible pattern thus formed is typically transferred to a receiver sheet and permanently affixed thereto.

Transfer processes of this type have several disadvantages where it is desired to reuse the photoconductor. If the image is developed with dry materials, the developing and transferring steps can result in considerable abrasion to the photoconductive surface. Abrasion is undesirable as it causes a reduction in image quality. If the electrostatic charge pattern is developed using liquid developers, the surface of the photoconductor often becomes coated with an uneven scum of dried developer. Unwanted deposits of this type adversely affect the electrical properties of the sensitive element. Attempts to remove these deposits may result in abrasion damage or solvent attack of the surface of the element.

Several means have been proposed for overcoming the problems described above. U.S. Pat. No. 2,975,052 discloses one of the simpler ways of avoiding these problems. The process of this patent is one wherein an electrostatic charge pattern is transferred from a photoconductive element to a receiving element having an electrically con-

## 2

ducting backing. During the transfer step the sensitive element and the receiving element are electrically connected or they are both grounded. In addition, the two elements are placed in close contact by the application of external pressure. This process, however, has several disadvantages in that it is somewhat slow in view of the fact that the two members must be suitably attached to electric connections, pressure applied and then the electrical connections broken.

- 10 A further disadvantage of the materials and process described in the above patent is that high resolutions are not attainable. In fact, when the invention is practiced according to the patent resolutions of only 30 to 60 lines per millimeter are obtained. Such low resolution capability makes such a process entirely unsuited where high resolution is required as, for example, in microimage recording and reproduction. According to "Microfilming of Engineering Documents, 35 mm.," Military Specification MIL-M-9868C, the minimum resolution requirement for Class I (negative camera microimage) at 16× reduction ratio is 101 line pairs/mm. At a 30× reduction ration, the minimum requirement is 120 line pairs/mm. Thus, it is readily apparent that a process which provides a resolution of only 60 lines per millimeter would be not be useful in forming Class I negative camera microimages.

Accordingly, there is a need in the art for a simple means of transferring electrostatic charge patterns, which means is rapid, simple and which allows the formation of high resolution images.

It is, therefore, an object of this invention to provide a novel means of transferring electrostatic charge patterns.

A further object of this invention is to provide a new method of transferring electrostatic charge patterns which is rapid and simple.

Another object of this invention is to provide a novel process for transferring and developing electrostatic charge patterns to obtain images of high resolution.

These and other objects and advantages of the invention are accomplished by the use of charge-image-bearing members and receiving elements having extremely smooth surfaces. In accordance with this invention, a charge pattern is formed on an image-bearing member which is then wetted with certain electrically insulating liquids. A smooth surfaced receiving element is then placed in contact with the wetted member and the charge pattern is transferred to the element without the application of any pressure or external electrical connections. The transferred pattern is then developed to form a visible image.

In accordance with this invention, an electrostatic charge pattern is produced on an image-bearing member by any of the suitable techniques known in the art of electrography. One particularly useful means of producing such charge patterns is by electrophotographic techniques. Electrophotography involves the use of a sensitive element typically comprising a conducting support having coated thereon a layer of a photoconductive composition.

Suitable supporting materials for use in elements of the type described above can include any of a wide variety of electrically conducting supports, for example, paper (at a relative humidity above 20 percent), aluminum foil-paper laminates; metal foils such as aluminum foil, zinc foil, etc.; metal plates, such as aluminum, copper, zinc, brass and galvanized plates; vapor deposited metal layers such as silver, nickel, aluminum and the like coated on paper or conventional photographic film bases such as cellulose acetate, polystyrene, poly(ethylene terephthalate), etc. Such conducting materials as nickel can be coated by vacuum deposition on transparent film supports in sufficiently thin layers to allow electrophotographic elements prepared therewith to be exposed from either side of such

elements. An especially useful conducting support can be prepared by coating a support material such as poly(ethylene terephthalate) with a conducting layer containing a semiconductor such as cuprous iodide dispersed in a resin. Such conducting layers both with and without insulating barrier layers are described in U.S. Pats. 3,245,833 and 3,428,451. Likewise, a suitable conducting coating can be prepared from the sodium salt of a carboxyester lactone of maleic anhydride and a vinyl acetate polymer. Such kinds of conducting layers and methods for their optimum preparation and use are disclosed in U.S. Pat. Nos. 3,007,901 and 3,267,807.

The photoconductive compositions which can be coated on the above supports include a wide variety of materials. Useful compositions typically comprise a photoconductive compound in an electrically insulating, film-forming resin binder. Both inorganic and organic photoconductors can be used in the present invention as well as mixtures of two or more photoconductors. Suitable inorganic photoconductors would include zinc oxide, cadmium sulfide, cadmium selenide, titanium dioxide and others. Useful organic photoconductors include the following materials.

(A) Arylamine photoconductors including substituted and unsubstituted arylamines, diarylamines, nonpolymeric triarylamines and polymeric triarylamines such as those described in U.S. Pats. 3,240,597 and 3,180,730.

(B) Photoconductors represented by the formula:



wherein Z represents a mononuclear or polynuclear divalent aromatic radical, either fused or linear (e.g., phenyl, naphthyl, biphenyl, binaphthyl, etc.), or a substituted divalent aromatic radical of these types wherein said substituent can comprise a member such as an acyl group having from 1 to about 6 carbon atoms (e.g., acetyl, propionyl, butyryl, etc.), an alkyl group having from 1 to about 6 carbon atoms (e.g., methyl, ethyl, propyl, butyl, etc.), an alkoxy group having from 1 to about 6 carbon atoms (e.g., methoxy, ethoxy, propoxy, pentoxy, etc.) or a nitro group; Z' represents a mononuclear or polynuclear monovalent or polynuclear monovalent aromatic radical, either fused or linear (e.g., phenyl, naphthyl, biphenyl, etc.); or a substituted monovalent aromatic radical wherein said substituent can comprise a member, such as an acyl group having from 1 to about 6 carbon atoms (e.g., acetyl, propionyl, butyryl, etc.), an alkyl group having from 1 to about 6 carbon atoms (e.g., methyl, ethyl, propyl, butyl, etc.), an alkoxy group having from 1 to about 6 carbon atoms (e.g., methoxy, propoxy, pentoxy, etc.), or a nitro group; Q can represent a hydrogen atom or an aromatic amino group, such as Z'NH<sup>-</sup>; b represents an integer from 1 to about 12, and L represents a hydrogen atom, a mononuclear or polynuclear aromatic radical, either fused or linear (e.g., phenyl, naphthyl, biphenyl, etc.), a substituted aromatic radical wherein said substituent comprises an alkyl group, an alkoxy group, an acyl group, or a nitro group, or a poly(4'-vinylphenyl) group which is bonded to the nitrogen atom by a carbon atom of the phenyl group, these materials being more fully described in U.S. Pat. 3,265,496.

(C) Polyarylalkane photoconductors including leuco bases of diaryl or triarylmethane dye salts, 1,1,1-triarylalkanes wherein the alkane moiety has at least two carbon atoms and tetraarylmethanes having an amino group substituted in at least one of the aryl nuclei attached to the alkane and methane moieties of the latter two classes of photoconductors which are non-leuco base materials; and also other polyarylalkanes includes by the formula:



wherein each of D, E and G is an aryl group and J is a hydrogen atom, an alkyl group, or an aryl group, at least one of D, E and G containing an amino substituent, the aryl groups attached to the central carbon atom being preferably phenyl groups, although naphthyl groups can also be used including substituted aryl groups containing substituents such as alkyl and alkoxy typically having 1 to 8 carbon atoms, hydroxy, halogen, etc., in the ortho, meta or para positions, ortho-substituted phenyl being preferred; the aryl groups can also be joined together or cyclized to form a fluorene moiety, for example; the amino substituent can be represented by the formula



wherein each R can be an alkyl group typically having 1 to 8 carbon atoms, a hydrogen atom, an aryl group, or together the necessary atoms to form a heterocyclic amino group typically having 5 to 6 atoms in the ring such as morpholino, pyridyl, pyrrolyl, etc.; at least one of D, E and G preferably being a p-dialkylaminophenyl group, when J is an alkyl group, such an alkyl group more generally has 1 to 7 carbon atoms, these materials being more fully described in U.S. Pat. 3,274,000, French Pat. 1,383,461 and in U.S. Ser. No. 627,857 filed Apr. 3, 1967 by Seus and Goldman.

(D) Photoconductors comprising 4-diarylamino substituted chalcones having the formula:



wherein R<sub>1</sub> and R<sub>2</sub> are each phenyl radicals including substituted phenyl radicals, R<sub>2</sub> preferably having the formula:



wherein R<sub>3</sub> and R<sub>4</sub> are each aryl radicals, aliphatic residues of 1 to 12 carbon atoms such as alkyl radicals preferably having 1 to 4 carbon atoms, or hydrogen; particularly advantageous results being obtained when R<sub>1</sub> is a phenyl radical including a substituted phenyl radical and where R<sub>2</sub> is diphenylaminophenyl, dimethylaminophenyl or phenyl, these materials being more fully described in Fox application U.S. Ser. No. 613,846, now U.S. Pat. 3,526,501.

(E) Non-ionic cycloheptenyl compounds which may be substituted with substituents such as:

- (1) an aryl radical including substituted as well as unsubstituted aryl radicals,
- (2) a hydroxy radical,
- (3) an azido radicals,
- (4) a heterocyclic radical having 5 to 6 atoms in the heterocyclic nucleus and at least one hereto nitrogen atom, and including substituted and unsubstituted heterocyclic radicals, and
- (5) an oxygen linked cycloheptenyl moiety.

The substitution on the cycloheptenyl nucleus occurs at an unsaturated carbon atom when the cycloheptenyl moiety is a conjugated triene with no aromatic structure fused thereto. However, if there is at least one aromatic structure fused to the cycloheptenyl moiety, then the substituents are attached to a saturated carbon atom. Additional photoconductors within this class are included in one of the following formulae:



where  $E_2$  and  $G_2$  can be either:

- (1) a phenyl radical,
- (2) a naphthyl radical,
- (3) a heterocyclic radical having 5 to 6 atoms in the heterocyclic nucleus and at least one hereto nitrogen atom,
- (4) a hydroxyl radical, or
- (5) an oxygen containing radical having a structure such that the resultant cycloheptenyl compound is a symmetrical ether;

$D_2$  can be any of the substituents defined for  $E_2$  and  $G_2$  above and is attached to a carbon atom in the cycloheptenyl nucleus having a double bond; ( $R_9$  and  $R_{10}$ ), ( $R_{11}$  and  $R_{12}$ ), ( $R_5$  and  $R_6$ ), and ( $R_7$  and  $R_8$ ) are together the necessary atoms to complete a benzene ring fused to the cycloheptenyl nucleus; these compounds being more fully described in U.S. Ser. No. 654,091 filed July 18, 1967, now U.S. Pat. 3,533,786.

(F) Compounds containing an  $>N-N<$  nucleus including:

- (1) unsubstituted and substituted N,N-bicarbazyls containing substituents in either or both carbazolyl nuclei such as:
  - (a) an alkyl radical including a substituted alkyl radical such as a haloalkyl or an alkoxyalkyl radical,
  - (b) a phenyl radical including a substituted phenyl radical such as a naphthyl, an aminophenyl or a hydroxyphenyl radical,
  - (c) a halogen atom,
  - (d) an amino radical including substituted as well as unsubstituted amino radicals such as an alkylamino or a phenylalkylamino radical,
  - (e) an alkoxy radical,
  - (f) a hydroxyl radical,
  - (g) a cyano radical,
  - (h) a heterocyclic radical such as a pyrazolyl, carbazolyl or a pyridyl radical; or
- (2) tetra-substituted hydrazines containing substituents which are substituted or unsubstituted phenyl radicals, or heterocyclic radicals having 5 to 6 atoms in the hetero nucleus, suitable results being obtained when all four substituents are not unsubstituted phenyl radicals, i.e., if at least one substituent is a substituted phenyl radical or a heterocyclic radical having 5 to 6 atoms in the hetero nucleus. Other tetra-substituted hydrazines include those having the following formula:



wherein  $D_1$ ,  $E_1$ ,  $G_1$  and  $J_1$  are each either:

- (a) a substituted phenyl radical such as a naphthyl radical, an alkyl phenyl radical, a halophenyl radical, a hydroxyphenyl radical, a haloalkylphenyl radical or a hydroxyalkylphenyl radical, or
- (b) a heterocyclic radical such as an imidazolyl radical, a furyl radical, or a pyrazolyl radical. In addition  $J_1$  and  $E_1$  can also be
- (c) an unsubstituted phenyl radical.

Especially preferred are those tetra-substituted hydrazines wherein both  $D_1$  and  $G_1$  are either substituted phenyl radicals or heterocyclic radicals. These compounds are more fully described in U.S. Ser. No. 673,962 filed Oct. 9, 1967.

(G) Organic compounds having a 3,3'-bis-aryl-2-pyrazoline nucleus which is substituted in either five-member ring with the same or different substituents. The 1 and 5 positions on both pyrazoline rings can be substituted by an aryl moiety including unsubstituted as well as substituted aryl substituents such as alkoxyaryl, alkaryl, alkaminoaryl, carboxyaryl, hydroxyaryl and haloaryl. The 4 position can contain hydrogen or unsubstituted as well as substituted alkyl and aryl radicals such as alkoxy-

aryl, alkaryl, alkaminoaryl, haloaryl, hydroxyaryl, alkoxy-alkyl, aminoalkyl, carboxyaryl, hydroxyalkyl and haloalkyl. Other photoconductors in this class are represented by the following structure:



wherein:

$D_3$ ,  $D_3'$ ,  $J_3$  and  $J_3'$  can be either a phenyl radical including a substituted phenyl radical such as a tolyl radical or a naphthyl radical including a substituted naphthyl radical,

$E_3$ ,  $E_3'$ ,  $G_3$ ,  $G_3'$ ,  $L_3$  and  $L_3'$  can be any of the substituents set forth above and in addition can be either a hydrogen atom or an alkyl radical containing 1 to 8 carbon atoms. These organic photoconductors are more fully described in U.S. Ser. No. 664,642 filed Aug. 31, 1967, now U.S. Pat. 3,527,602.

(H) Triarylamines in which at least one of the aryl radicals is substituted by either a vinyl radical or a vinylene radical having at least one active hydrogen-containing group. The phrase "vinylene radical" includes substituted as well as unsubstituted vinylene radicals and also includes those radicals having at least one and as many as three repeating units of vinylene groups such as



wherein  $n$  is an integer of from 1 to 3. Groups which contain active hydrogen are well known in the art, the definition of this term being set forth in several textbooks such as "Advanced Organic Chemistry," R. C. Fuson, pp. 154-157, John Wiley & Sons, 1950. The term "active hydrogen-containing group" as used herein includes those compounds encompassed by the discussion in the text book cited above and in addition includes those compounds which contain groups which are hydrolyzable to active hydrogen-containing groups. Typical active hydrogen-containing groups substituted on the vinylene radical of the triarylamine include:

- (1) carboxy radicals,
- (2) hydroxy radicals,
- (3) ethynyl radicals,
- (4) ester radicals (e.g.,



wherein  $R_{13}$  is alkyl or aryl) including cyclic ester radicals (e.g.,



wherein  $R_{14}$  is a cyclic alkylene radical connected to a vinylene combination such as is found in coumarin derivatives),

- (5) carboxylic acid anhydride radicals,
- (6) semicarbazono radicals,
- (7) cyano radicals,
- (8) acyl halide radicals (e.g.,



etc.), and

- (9) amido radicals (e.g.,



wherein  $R_{15}$  is a hydrogen atom, an alkyl group or an aryl group).

Other active hydrogen-containing groups include substituted and unsubstituted alkylidyne oximido radicals. Photoconductors included in this class can be represented by the following structure:



wherein:

- (1)  $\text{Ar}_1$  and  $\text{Ar}_2$  are each a phenyl radical including a substituted phenyl radical such as a halophenyl radical, an alkyl phenyl radical or an aminophenyl radical,
- (2)  $\text{Ar}_3$  is an arylene radical including a substituted arylene radical such as a phenylene radical or a naphthylene radical,
- (3)  $\text{R}_{16}$  and  $\text{R}_{17}$  are each hydrogen, a phenyl radical including a substituted phenyl radical or a lower alkyl radical preferably having 1 to 8 carbon atoms,
- (4)  $\text{X}$  is either:
  - (a) an active hydrogen-containing group such as a carboxy radical, an acyl halide radical, an amido radical, a carboxylic acid anhydride radical, an ester radical, a cyano radical, a hydroxy radical, a semicarbazono radical, an ethynyl radical, or a methylidyne oximido radical, or
  - (b) hydrogen, provided that when  $\text{X}$  is hydrogen  $\text{R}_{16}$  and  $\text{R}_{17}$  are also hydrogen, and
- (5)  $n$  is an integer of one to three.

The arylene nucleus can be substituted in any position by the vinyl or vinylene moiety. However, when  $\text{Ar}_3$  is phenylene, particularly good results are obtained if the substitution occurs in the para position. These materials are more fully described in U.S. Ser. No. 706,800 filed Feb. 20, 1968, now U.S. Pat. 3,567,450.

(I) Triarylamines in which at least one of the aryl radicals is substituted by an active hydrogen-containing group. The term "active hydrogen-containing group" has the same meaning as set forth above and again includes those compounds encompassed by the discussion in the textbook and additionally includes those compounds which contain groups which are hydrolyzable to active hydrogen-containing groups. Typical active hydrogen-containing groups which are substituted on an aryl radical of the triarylamine include:

- (1) carboxy radicals,
- (2) hydroxy radicals,
- (3) ethynyl radicals,
- (4) ester radicals (e.g.,



- wherein  $\text{R}_{18}$  is an alkyl or an aryl group),
- (5) lower alkylene hydroxy radicals (e.g., having 1 to 8 carbon atoms),
  - (6) carboxylic acid anhydride radicals,
  - (7) lower alkylene carboxy radicals (e.g., having 2 to 8 carbon atoms),
  - (8) cyano radicals,
  - (9) acyl halide radicals (e.g.,



- etc.),
- (10) amido radicals (e.g.,



wherein  $\text{R}_{19}$  is a hydrogen atom, an alkyl group or an aryl group),

(11) lower alkylidyne oximido radicals having 1 to 8 carbon atoms including substituted alkylidyne oximido radicals (e.g.,



wherein  $\text{R}_{20}$  is hydrogen or a lower alkyl radical),

(12) semicarbazono radicals, and

(13) arylene carboxy radicals including substituted arylene carboxy radicals (e.g.,



wherein  $\text{D}_4$  and  $\text{E}_4$  are phenyl or lower alkyl radicals).

Photoconductors included in this class can be represented by the following structure:



wherein:

- (a)  $\text{Ar}_4$  and  $\text{Ar}_5$  are each a phenyl radical including a substituted phenyl radical such as a halophenyl radical, an alkyl phenyl radical or an amino phenyl radical,
- (b)  $\text{Ar}_6$  is an arylene radical including a substituted arylene radical such as a phenylene radical or a naphthylene radical, and
- (c)  $\text{X}_1$  is an active hydrogen-containing group such as a carboxy radical, an acyl halide radical, an amido radical, a carboxylic acid anhydride radical, an ester radical, a cyano radical, a semicarbazono radical, a hydroxy radical, an ethynyl radical, a methylidyne oximido radical or a phenylene carboxy radical.

These materials are more fully described in U.S. Ser. No. 706,780 filed Feb. 20, 1968.

(J) Organo-metallic compounds having at least one amino-aryl substituent attached to a Group IVa or Group Va metal atom. The metallic substituents of this class of organic photoconductors are Group IVa or Group Va metals in accordance with the Periodic Table of the Elements (Handbook of Chemistry and Physics, 38th edition, pp. 394-95) and include silicon, germanium, tin and lead from Group IVa and phosphorus, arsenic, antimony and bismuth from Group Va. These materials can be substituted in the metallo nucleus with a wide variety of substituents but at least one of the substituents must be an amino-aryl radical. The amino radical can be positioned anywhere on the aromatic nucleus, but best results are obtained if the aryl moiety is a phenyl radical having the amino group in the 4 or para position. Typical substituents attached to the metal nucleus include the following:

- (1) a hydrogen, sulfur or oxygen atom,
- (2) an alkyl radical,
- (3) an aryl radical including unsubstituted as well as substituted aryl radicals such as aminoaryl, alkylaryl and haloaryl,
- (4) an oxygen-containing radical such as an alkoxy or aryloxy radical,
- (5) an amino radical including unsubstituted and substituted amino radicals such as mono- and diarylamino and mono- and dialkylamino radicals,
- (6) a heterocyclic radical, and
- (7) a Group IVa or Va organo-metallic radical.

Photoconductors included in this class can be represented by the following structures:



9



where  $E_5$ ,  $G_5$ ,  $L_5$  and  $Q_5$  can be:

- (a) a hydrogen atom,
- (b) an aryl radical including unsubstituted as well as substituted aryl radicals such as a phenyl radical, a naphthyl radical, a dialkylaminophenyl radical, or a diarylaminophenyl radical,
- (c) an alkyl radical having 1 to 8 carbon atoms,
- (d) an alkoxy radical having 1 to 8 carbon atoms,
- (e) an aryloxy radical such as a phenoxy radical,
- (f) an amino radical having the formula



wherein  $R_{21}$  and  $R_{22}$  can be hydrogen atoms or alkyl radicals having 1 to 8 carbon atoms, or

(g) a heterocyclic radical having 5 to 6 atoms in the hetero nucleus including at least one nitrogen atom such as a triazolyl, a pyridyl radical, etc.,

$T$  is an amino radical such as an alkylamino radical having 1 to 8 carbon atoms or an arylamino radical such as a phenylamino radical;

$Ar$  is an aromatic radical such as phenyl or naphthyl;

$M_{a1}$  and  $M_{a2}$  are the same or different Group IVa metals;

$M_b$  is a Group Va metal;

$D_5$  can be any of the substituents set forth above for  $E_5$ ,  $G_5$ ,  $L_5$  and  $Q_5$  and in addition can be a Group IVa organo-metallic radical or, when taken with  $E$ , an oxygen atom or a sulfur atom;

$J_5$  can be any of the substituents set forth above for  $E_5$ ,  $G_5$ ,  $L_5$  and  $Q_5$  and in addition can be when taken with  $E$ , an oxygen atom or a sulfur atom. These materials are described in U.S. Ser. No. 650,664, filed July 3, 1967.

(K) Any other organic compound which exhibits photoconductive properties such as those set forth in Australian Pat. 248,402.

Representative organic photoconductors useful in this invention include the compounds listed below:

TABLE I

diphenylamine  
dinaphthylamine  
 $N,N'$ -diphenylbenzidine  
 $N$ -phenyl-1-naphthylamine  
 $N$ -phenyl-2-naphthylamine  
 $N,N'$ -dihphenyl-p-phenylenediamine  
2-carboxy-5-chloro-4'-methoxydiphenylamine  
p-anilinophenol  
 $N,N'$ -di-2-naphthyl-p-phenylenediamine  
4,4'-benzylidene-bis-( $N,N$ -dimethyl-m-toluidine)  
triphenylamine  
 $N,N,N',N'$ -tetraphenyl-m-phenylenediamine

- 4-acetyltriphenylamine  
4-hexanoyltriphenylamine  
4-lauroyltriphenylamine  
4-hexyltriphenylamine  
5 4-dodecyltriphenylamine  
4,4'-bis(diphenylamino)benzil  
4,4'-bis(diphenylamino)benzophenone  
poly[N,4''-( $N,N,N'$ -triphenylbenzidine)]  
polyadipyltriphenylamine  
polysebacyltriphenylamine  
polydecamethylenetriphenylamine  
poly-N-(4-vinylphenyl)diphenylamine  
poly-N-(vinylphenyl)- $\alpha,\alpha'$ -dinaphthylamine  
4,4'-benzylidene-bis( $N,N$ -diethyl-m-toluidine)  
15 4',4''-diamino-4-dimethylamino-2',2''-dimethyltriphenylmethane  
4',4''-bis(diethylamino)-2,6-dichloro-2,2''-dimethyltriphenylmethane  
4',4''-bis(diethylamino)-2',2''-dimethyldiphenylmethane  
20 2',2''-dimethyl-4,4',4''-tris(dimethylamino)triphenylmethane  
4',4''-bis(diethylamino)-4-dimethylamino-2',2''-dimethyltriphenylmethane  
25 4',4''-bis(diethylamino)-2-chloro-2',2''-dimethyl-4-dimethylaminotriphenylmethane  
4',4''-bis(diethylamino)-4-dimethylamino-2',2''-trimethyltriphenylmethane  
4',4''-bis(dimethylamino)-2-chloro-2',2''-dimethyltriphenylmethane  
30 35 4',4''-bis(dimethylamino)-2',2''-dimethyl-4-methoxytriphenylmethane  
bis(4-diethylamino)-1,1,1-triphenylethane  
bis(4-diethylamino)tetraphenylmethane  
4',4''-bis(benzylethylamino)-2',2''-dimethyltriphenylmethane  
4',4''-bis(diethylamino)-2',2''-diethoxytriphenylmethane  
4,4'-bis(dimethylamino)-1,1,1-triphenylethane  
1-(4-N,N-dimethylaminophenyl)-1,1-diphenylethane  
40 4-dimethylaminotetraphenylmethane  
4-diethylaminotetraphenylmethane  
4,4'-bis(diphenylamino)chalcone  
4-diphenylamino-4'-dimethylaminochalcone  
4-dimethylamino-4'-diphenylaminochalcone  
4,4'-bis(dimethylamino)chalcone  
45 50 4,4'-bis(diethylamino)chalcone  
4-diethylamine-4'-diphenylaminochalcone  
4-diphenylaminochalcone  
4-dimethylaminochalcone  
4'-diphenylaminochalcone  
4-dimethylaminochalcone  
bis-[5-(5H-dibenzo[a,d]cycloheptenyl)]ether  
5-hydroxy-5H-dibenzo[a,d]cycloheptene  
1-{5-(5H-dibenzo[a,d]cycloheptenyl)}-4,5-dicarboxy-1,2,3-triazole  
55 1-{5-(5H-dibenzo[a,d]cycloheptenyl)}-4,5-dibenzoyl-1,2,3-triazole  
5-azido-5H-dibenzo[a,d]cycloheptene  
1-{5-(10,11-dihydro-5H-dibenzo[a,d]cycloheptenyl)}-4,5-dicarbomethoxy-1,2,3-triazole  
60 1-{5-(10,11-dihydro-5H-dibenzo[a,d]cycloheptenyl)}-4,5-dibenzoyl-1,2,3-triazole  
4-[5-(5H-dibenzo[a,d]cycloheptenyl)]-N,N-dimethylaniline  
N,N-diethyl-3-methyl-4-[5-(5H-dibenzo[a,d]cycloheptenyl)]aniline  
65 4-[5-(5H-dibenzo[a,d]cycloheptenyl)]-1-dimethylamino-naphthalene  
N,N-diethyl-3-methyl-4-[5-(10,11-dihydro-5H-dibenzo[a,d]cycloheptenyl)]aniline  
70 3-(4-dimethylaminophenyl)-1,3,5-cycloheptatriene  
3-(4-diethylamino-2-methylphenyl)-1,3,5-cycloheptatriene  
3-(4-dimethylaminonaphthyl)-1,3,5-cycloheptatriene  
N,N-diethyl-3-methyl-4-[5-(5H-dibenzo[a,d]cycloheptenyl)]aniline  
75

tetra- $\alpha$ -naphthylhydrazine  
 tetra(3-methyl-4-hydroxyphenyl)hydrazine  
 tetra(m-hydroxyethylphenyl)hydrazine  
 tetra(2-methyl-5-chloroethylphenyl)hydrazine  
 tetra(2-methyl-5-hydroxyphenyl)hydrazine  
 tetra(1-imidazolyl)hydrazine  
 N,N-di- $\alpha$ -naphthyl-N',N'-di(3-methyl-4-hydroxyphenyl)hydrazine  
 N-3-furyl-N-(2-methyl-4-hydroxyphenyl)-N',N'-di- $\beta$ -naphthylhydrazine  
 tetra- $\beta$ -naphthylhydrazine  
 N,N'-di- $\beta$ -naphthyl-N,N'-diphenylhydrazine  
 tetra-4-tolylhydrazine  
 N,N'-diphenyl-N,N'-di(3-methyl-4-hydroxyphenyl)hydrazine  
 N,N'-diphenyl-N,N'-di-p-chlorophenyl hydrazine  
 phenyltri-(2-methyl-5-hydroxyphenyl)hydrazine  
 N,N'-bicarbazyl  
 cyclotetrakis(3,9-carbazolylene)  
 6-(3-carbazolyl)cyclotetrakis(3,9-carbazolylene)  
 6-(3-carbazolyl)-cyclotetrakis(3,9-carbazolylene)  
 3,3'-bis(3-carbazolyl)-9,9'-bicarbazolyl  
 3-(3-carbazolyl)-9-(9-carbazolyl)carbazole  
 3-(9-carbazolyl)-9,9'-bicarbazolyl  
 3,3'-diethyl-9,9'-bicarbazolyl  
 3,3'-diphenyl-9,9'-bicarbazolyl  
 3,3'-dichloro-9,9'-bicarbazolyl  
 4,4'-bis(diethylamino)-9,9'-bicarbazolyl  
 3,3'-diethoxy-9,9'-bicarbazolyl  
 1,1'-dihydroxy-9,9'-bicarbazolyl  
 2,2'-dicyano-9,9'-bicarbazolyl  
 tetra(p-diethylaminophenyl)hydrazine  
 3,3'-bis(1,5-diphenyl-2-pyrazoline)  
 3,3'-bis(1-p-tolyl-5-phenyl-2-pyrazoline)  
 3,3'-bis(1,5-[1-naphthyl]-2-pyrazoline)  
 1,5-diphenyl-3-[3'-(1'-p-tolyl-5'-phenyl)-2'-pyrazolyl]-2-pyrazoline  
 3,3'-bis(1,5-diphenyl-4,5-dimethyl-2-pyrazoline)  
 3,3'-bis(1,4,5-triphenyl-2-pyrazoline)  
 3,3'-bis(1,5-di-p-tolyl-4-methoxy-2-pyrazoline)  
 3,3'-bis(1,5-diphenyl-4-dimethylamino-2-pyrazoline)  
 3,3'-bis[1,5-diphenyl-4-(p-chlorophenyl)-2-pyrazoline]  
 3,3'-bis[1,5-diphenyl-4,5-di-(p-diethylaminophenyl)-2-pyrazoline]  
 3,3'-bis[1,5-diphenyl-4-(p-methoxyphenyl)-5-ethyl-2-pyrazoline]  
 3,3'-bis(1,5-diphenyl-4-chloromethyl-2-pyrazoline)  
 1,5-diphenyl-4,5-dimethyl-3-[3'-(1'-p-tolyl-4-diethyl-5,5'-methylphenyl)-2'-pyrazolyl]-2-pyrazoline  
 4-(p-diphenylaminophenyl)-3-buten-1-yne  
 p-diphenylaminostyrene  
 ethyl p-diphenylaminocinnamate  
 methyl p-diphenylaminocinnamate  
 p-diphenylaminocinnamoyl chloride  
 p-diphenylaminocinnamic acid N,N-diphenylamide  
 p-diphenylaminocinnamic acid anhydride  
 3-(p-diphenylaminophenyl)-2-butenoic acid  
 bis(p-diphenylaminobenzyl)succinic acid  
 4-N,N-bis(p-bromophenyl)aminocinnamic acid  
 1-(4-diphenylamino)naphthacrylic acid  
 p-diphenylaminocinnamic acid  
 p-diphenylaminocinnamontitrile  
 7-diphenylaminocoumarin  
 p-diphenylaminophenylvinylacrylic acid  
 p-diphenylaminobenzyl p'-diphenylaminocinnamate  
 7-(p-diphenylaminostyryl)coumarin  
 p-diphenylaminocinnamyl alcohol  
 4-diphenylaminocinnamaldehyde semicarbazone  
 O-p-diphenylaminocinnamoyl p'-diphenylaminobenzaldehyde oxime  
 p-diphenylaminocinnamaldehyde oxime  
 1,3-bis(p-diphenylaminophenyl)-2-propen-1-ol  
 methyl p-diphenylaminobenzoate  
 N,N-diphenylanthranilic acid  
 3-p-diphenylaminophenyl-1-propanol

4-acetyltriphenylamine semicarbazone  
 ethyl 2,6-diphenyl-4-(p-diphenylaminophenyl)benzoate  
 1-(p-diphenylaminophenyl)-1-hydroxy-3-butyne  
 4-hydroxymethyltriphenylamine  
 5 1-(p-diphenylaminophenyl)ethanol  
 4-hydroxytriphenylamine  
 2-hydroxytriphenylamine  
 4-formyltriphenylamine oxime  
 4-acetyltriphenylamine oxime  
 10 1-(p-diphenylaminophenyl)hexanol  
 1-(p-diphenylaminophenyl)dodecanol  
 p-diphenylaminobenzoic acid anhydride  
 4-cyanotriphenylamine  
 p-diphenylaminobenzoic acid N,N-diphenylamide  
 15 p-diphenylaminobenzoic acid  
 p-diphenylaminobenzoyl chloride  
 3-p-diphenylaminophenylpropionic acid  
 4-formyltriphenylamine semicarbazone  
 triphenyl-p-diethylaminophenylsilane  
 20 methyl-diphenyl-p-diethylaminophenylsilane  
 triphenyl-p-diethylaminophenylgermane  
 triphenyl-p-dimethylaminophenylstannane  
 triphenyl-p-diethylaminophenylstannane  
 diphenyl-di-(p-diethylaminophenyl)stannane  
 25 triphenyl-p-diethylaminophenylplumbane  
 tetra-p-diethylaminophenylplumbane  
 phenyl-di-(p-diethylaminophenyl)phosphine  
 bis(p-diethylaminophenyl)phosphine oxide  
 tri-p-dimethylaminophenylarsine  
 30 tri-p-diethylaminophenylarsine  
 2-methyl-4-dimethylaminophenylarsine oxide  
 tri-p-diethylaminophenylbismuthine  
 methyl-di-(p-diethylaminophenyl)arsine  
 methyl-di-(p-diethylaminophenyl)phosphine  
 35 phenyl-tri-(p-diethylaminophenyl)stannane  
 methyl-tri-(p-diethylaminophenyl)stannane  
 tetra-p-diethylaminophenylgermane  
 diphenyl-p-diethylaminophenylsilane  
 p-diethylaminophenylarsine  
 40 tetrakis-[diphenyl-(p-diethylaminophenyl)plumbyl]  
 methane  
 tetrakis-[diphenyl-(p-diethylaminophenyl)stanny]  
 stannane  
 bis[phenyl-(p-diethylaminophenyl)]dibismuthine  
 tri(p-diethylaminophenyl)phosphine sulfide  
 45 di-(p-diethylaminophenyl)thioxotin

Photoconductive compositions of the type described above can be sensitized, if so desired, with any of the sensitizing materials now well known in the art.

50 The image-bearing members whether comprised simply of a sheet of insulating material or in the form of an electrophotographic element, all have in common an extremely smooth surface to which the electrostatic charge pattern is applied. In general, the image-bearing member has a Sheffield Smoothness value in the range of about 0 to 25 with preferred materials having a value in the range of about 0 to 10. Sheffield Smoothness value is a measure of smoothness which conforms to TAPPI Standard No. T-479SM48. The equipment utilized in making the smoothness measurements is made by the Sheffield Corporation of Dayton, Ohio. Briefly, the components of the equipment are (I) a precision device in which a sheet sample is held against a smooth glass plate under an accurately weighed, precision-machined head through which a regulated stream of air flows, and (II) a Modular-Precisionaire Instrument which measures the flow of air across the face of the sheet sample. Data are read in numerical units from 0 for extreme smoothness to 400 for rough surfaces.

65 In general, the sensitive elements of the type described above can be employed in any of the well known electrophotographic processes which require photoconductive layers. In one process of this type, an electrophotographic element is held in the dark and given a blanket electro-

static charge by placing it under a corona discharge. This uniform charge is retained by the sensitive layer because of the substantial dark insulating property of the layer, i.e., the low conductivity of the layer in the dark. The electrostatic charge formed on the surface of the photoconductive is then selectively dissipated from the surface of the layer by imagewise exposure to light by means of a conventional exposure operation such as, for example, by a contact-printing technique, or by lens projection of an image, and the like, to thereby form an electrostatic latent image in the photoconductive layer. Exposing the surface in this manner forms a pattern of electrostatic charge by virtue of the fact that light energy striking the photoconductor causes the electrostatic charge in the light struck areas to be conducted away from the surface in proportion to the intensity of the illumination in a particular area.

Now in accordance with the present invention, the smooth surface of the image-bearing member is wetted with an electrically insulating particle-free transfer liquid. This liquid can be applied by any suitable means such as spraying, pouring, swabbing, squeegeeing, immersion and the like. Useful materials for wetting the image-bearing member include hydrocarbon liquids typically having a boiling point in the range of about 105 to 260° C. and a volume resistivity of at least about  $10^{12}$  ohm-cm. The transfer liquids should exhibit no substantial solvent action on either the image-bearing member or the receiving element. Similarly, the transfer liquid should be compatible with any liquid developing materials used to develop the transferred charge pattern. Included among the preferred transfer liquids are isoparaffinic hydrocarbons having a low dielectric constant preferably below about 2.5. Specific liquids which are useful include various solvents made by Humble Oil & Refining Co. and sold under the trade name of Isopar, such as Isopar C, Isopar E, Isopar G, Isopar H, Isopar K, Isopar L, Isopar M, etc. Mixtures of suitable liquids can also be utilized.

After application of the transfer liquid, the receiving element can be immediately placed in contact with the wetted member. However, to insure a uniform thickness of liquid over the whole surface of the element, it is often desirable to allow the liquid to partially dry for a brief period. The liquid layer can also be rapidly wiped with a squeegee or similar device to insure a uniform thickness of the liquid layer. The process of this invention can be rapidly accomplished without the drying or squeegeeing steps; however, these steps insure a greater degree of reproducibility.

The receiving elements useful in the present invention can be formed of a variety of sheet materials. Suitable receiving elements have an electrically insulating layer and an electrically conductive backing or support. These elements are preferably flexible and all have in common at least one electrically insulating surface which typically has a resistivity of at least about  $10^{11}$  ohm-cm. and which is extremely smooth. In general, this surface of the element has a Sheffield Smoothness value, as described above, in the range of 0 to 25 with preferred materials having a value in the range of 0 to 10. Useful receiving elements can be formed using a variety of different conducting supports, for example, paper (at a relative humidity above 20 percent), aluminum foil-paper laminates; metal foils, such as aluminum foil, zinc foil, etc.; vapor deposited metal layers such as silver, nickel, aluminum and the like coated on paper or conventional photographic film bases such as cellulose acetate, polystyrene, poly(ethylene terephthalate), etc. Such conducting materials as nickel can be coated by vacuum deposition on transparent film supports in sufficiently thin layers as to result in a transparent element. An especially useful conducting support can be prepared by coating a support material such as poly(ethylene terephthalate) with a conducting layer containing a semiconductor such as cuprous iodide dispersed in a resin. Such conducting layers are described in U.S. Pats.

3,245,833 and 3,428,451. In addition, a suitable conducting coating can be prepared from the sodium salt of a carboxyester lactone of maleic anhydride and a vinyl acetate polymer. Conducting layers of this latter type and methods for their preparation and use are described in U.S. Pat. Nos. 3,007,901 and 3,267,807.

The conducting support is then overcoated with a suitable electrically insulating resin to provide the requisite extremely smooth surface. Suitable resins for this purpose can include any of a wide variety of electrically insulating, film-forming resins. Typical resins useful in this invention would include polyesters, polyolefins, such as polyethylene and polypropylene, polycarbonates, polyamides, poly(alkyl methacrylates) and the like. Mixtures of various resins can be used as well as plasticized resins. The only requirements of the resins used are that they be electrically insulating, film-forming, reasonably flexible and capable of being coated so as to have the requisite surface smoothness. The receiving element can be opaque or transparent depending upon the type of final image desired.

The receiving element can, of course, be wetted with the transfer liquid and then placed in contact with a dry image-bearing member. Regardless of which is wetted first, the member and element are always placed in face to face contact in the presence of an intermediate layer of transfer liquid. Intimate contact of the member and element is obtained without the application of any external pressure. In addition, no forward or reverse bias potentials are applied between the image-bearing member and the receiving element before, during or after transfer of the charge pattern. Also, the member and element do not have to be electrically grounded during transfer.

When the extremely smooth elements of the type described herein are used in the present process, which involves a thin layer of transfer liquid, resolutions of at least 135 line pairs per millimeter are obtainable. In a particularly preferred embodiment of the invention, the layer of transfer liquid is squeegeed, is allowed to partially dry or is otherwise treated or applied such that the layer is extremely thin, probably having a thickness in the range of about 1 to 5 microns. In this latter instance, images are obtainable which have a resolution of at least about 150 lines/mm.

The following examples are included for a further understanding of the invention.

#### EXAMPLE 1

An electrophotographic element is prepared by coating a layer of poly(vinyl-m-bromobenzoate-co-vinyl acetate) containing about 25% by weight of 4,4'-diethylamino-2,2'-dimethyltriphenylmethane photoconductor onto a conductive support comprising a cuprous iodide conducting layer on a poly(ethylene terephthalate) film base which is coated with a terpolymer of itaconic acid, ethyl acrylate and vinylidene chloride. The conducting layer is overcoated with a barrier layer of cellulose nitrate. The photoconductive layer is coated at a wet thickness of 0.004 inch. The coating is allowed to dry at room temperature and further dried by placing the element in a hot-air oven with an air temperature of about 60° C. After complete drying, the element is examined and found to have an extremely smooth surface on the photoconductive layer. The Sheffield Smoothness value of this surface is about 5. This element is then charged using a negative corona source until the surface potential reaches a value of minus 700 volts. The charged element is then exposed to a negative-appearing microimage having a maximum density of 1.5 and a maximum resolution of 160 line-pairs per millimeter. The exposure is made using an 85-watt Mercury light source. The exposed element is then placed in contact with a receiving element comprising a poly(ethylene terephthalate) film base having a cuprous iodide conducting layer which is overcoated with an ex-

## 15

tremely smooth-surfaced resin layer of poly(vinyl-m-bromobenzoate-covinyl acetate). The receiving element is then peeled away from the image-bearing member and immersed in a liquid developer comprising an isoparaffinic hydrocarbon carrier liquid having dispersed therein marking particles comprised of phenol formaldehyde resin, soya modified alkyd resin and carbon black. The resulting image has a maximum density of about 1.5 and a resolution of approximately 100 line-pairs per millimeter.

## EXAMPLE 2

The procedure of Example 1 is repeated except the receiver sheet used is comprised of insulating coating of Polyester 49,000 on a cuprous iodide coated poly(ethylene terephthalate) film base. Polyester 49,000 is a polyester obtained from Du Pont Co. and is prepared from ethylene glycol and equal amounts of dimethyl terephthalate and dimethyl isophthalate with small amounts of adipic and sebatic acids. The element is charged, exposed and developed as in Example 1 and found to have similar resolution but with lower maximum density.

## EXAMPLE 3

The procedure of Example 1 is repeated several times only using an electrical potential between the conductive layer of the receiving element and the conductive layer of the photoconductive element. Forward bias potentials of from 225 to 1000 volts are used during the transfer operation with the receiving element being positive with respect to the photoconductive element. The resulting images are similar to those obtained in Example 1 with no significant change in resolution. However, unwanted density is obtained in the background image areas.

## EXAMPLE 4

The procedure of Example 3 is repeated using a reverse bias potential of 225 volts during transfer with the receiving element at a negative polarity. After development, the resulting image is found to have a lower resolution with only 60 line-pairs per millimeter being obtainable.

## EXAMPLE 5

The procedure of Example 1 is generally followed except that, after exposure, the photoconductive film is wetted by dipping it into a bath of Isopar G. Isopar G is an isoparaffinic hydrocarbon solvent having a boiling point in the range of 150 to 185° C. (Humble Oil & Refining Co.). The wetted image-bearing member is placed in contact with a receiving element as before and the receiving element is then carefully peeled away and developed as in Example 1. During the transfer operation, no external pressure or electrical bias potentials are applied. After developing the transferred charge image, the resolution is found to be 135 line-pairs per millimeter.

## EXAMPLE 6

The procedure in Example 5 is repeated entirely except that the receiving element is first wetted and then placed in contact with the dry image-bearing member. Similar results are obtained.

## EXAMPLE 7

The procedure of Example 6 is repeated entirely except the receiver surface is allowed to dry partially for a period of 1 minute after being immersed in the transfer liquid. The partially dried receiver element is then placed in contact with the image-bearing member and carefully peeled away. The resulting image has a higher and more uniform maximum density and has a resolution of at least 150 line-pairs per millimeter.

## EXAMPLE 8

The procedure of Example 5 is repeated several times using electrical bias potentials in the range of about 500

## 16

and 1200 volts with the conductive layer of the receiving element being positive and that of the image-bearing member being negative. This results in an increased maximum density; however, it also results in an increased minimum density above the desirable level. In addition, the resolution is adversely affected.

## EXAMPLE 9

The procedure of Example 5 is followed again only in place of the isoparaffinic hydrocarbon transfer liquid, Dow Corning Fluid 200 Silicon Oil is used, which oil has a viscosity of about 2 centistokes. The resulting image has a resolution considerably below that obtained in Example 5.

The invention has been described in detail with particular reference to certain preferred embodiments thereof, but it will be understood that variations and modifications can be effected within the spirit and scope of the invention.

I claim:

1. A high resolution process for transferring an electrostatic charge pattern formed on a member capable of retaining an electrostatic charge pattern having a Sheffield Smoothness value of about 0 to 25 to a receiving element which is electrically insulating, has a resistivity of at least about  $10^{11}$  ohm-cm. has a Sheffield Smoothness value of about 0 to 25 and developing such transferred charge pattern, said process comprising the steps of:

(a) applying to one of said member and receiving element an electrically insulating isoparaffinic hydrocarbon transfer liquid having a boiling point in the range of about 105 to about 260° C. and a volume resistivity of at least about  $10^{12}$  ohm-cm.,

(b) placing said member and said element in face-to-face contact in the presence of said transfer liquid,

(c) transferring said charge pattern from said member to said element in the absence of external pressure and electrical bias potential, and

(d) developing said transferred charge pattern to produce an image having a resolution of at least about 100 lines/mm.

2. A high resolution process for transferring an electrostatic charge pattern formed on a member capable of retaining an electrostatic charge pattern having a Sheffield Smoothness value of about 0 to 25 to a receiving element which is electrically insulating, has a resistivity of at least about  $10^{11}$  ohm-cm. and has a Sheffield Smoothness value of about 0 to 25 and developing such transferred charge pattern, said process comprising the steps of:

(a) applying to said member an electrically insulating isoparaffinic hydrocarbon transfer liquid having a boiling point in the range of about 105 to about 260° C. and a volume resistivity of at least about  $10^{12}$  ohm-cm.,

(b) placing said member and said element in face-to-face contact in the presence of said transfer liquid,

(c) transferring said charge pattern from said member to said element in the absence of external pressure and electrical bias potential, and

(d) developing said transferred charge pattern to produce an image having a resolution of at least about 135 lines/mm.

3. A high resolution process for transferring an electrostatic charge pattern formed on a member capable of retaining an electrostatic charge pattern having a Sheffield Smoothness value of about 0 to 25 to a receiving element which is electrically insulating, has a resistivity of at least about  $10^{11}$  ohm-cm. and has a Sheffield Smoothness value of about 0 to 25 and developing such transferred charge pattern, said process comprising the steps of:

(a) applying to one of said member and receiving element an electrically insulating isoparaffinic hydrocarbon transfer liquid having a boiling point in the

- range of about 105 to about 260° C. and a volume resistivity of at least about  $10^{12}$  ohm-cm.,  
 (b) treating said applied transfer liquid to form a layer having a thickness between 1 to 5 microns,  
 (c) placing said member and said element in face-to-face contact in the presence of said transfer liquid,  
 (d) transferring said charge pattern from said member to said element in the absence of external pressure and electrical bias potential, and  
 (e) developing said transferred charge pattern to produce an image having a resolution of at least about 150 lines/mm.

4. A process as described in claim 1 including the further step of allowing said liquid to partially dry prior to contact with said receiving element.

5. A process as described in claim 1 wherein said member is an electrophotographic element bearing a light-sensitive layer containing an organic photoconductor.

6. A process as described in claim 1 wherein said transferred charge pattern is developed with a liquid developer compatible with said isoparaffinic hydrocarbon transfer liquid.

7. A process as described in claim 1 wherein said transfer liquid has no substantial solvent action on the member and the receiving element.

8. A process as described in claim 3 wherein said member is an electrophotographic element bearing a layer containing an organic photoconductor.

9. A process as described in claim 3 wherein the surface of said receiving element which bears the trans-

ferred charge is electrically insulating and has a resistivity of at least about  $10^{11}$  ohm-cm.

10. A process as described in claim 3 wherein said liquid developer is a liquid developer comprised of marking particles dispersed in a carrier liquid which is compatible with said transfer liquid.

11. A process as described in claim 3 wherein said applied liquid is allowed to partially dry.

12. A process as described in claim 3 wherein said applied liquid is subjected to a squeegeeing treatment to form a uniform thin layer of liquid.

13. A process as described in claim 3 wherein the gap between said member and said element during transfer is about 1 to 5 microns.

#### References Cited

##### UNITED STATES PATENTS

|           |         |                      |        |
|-----------|---------|----------------------|--------|
| 2,975,052 | 3/1961  | Fotland et al. ----- | 96—1   |
| 3,539,255 | 11/1970 | Goffe -----          | 96—1 X |
| 2,937,943 | 5/1960  | Walkup -----         | 96—1   |
| 3,394,002 | 7/1968  | Bickmore -----       | 96—1   |
| 2,833,648 | 5/1958  | Walkup -----         | 96—1   |
| 3,356,498 | 12/1967 | Moe et al. -----     | 96—1   |

23 CHARLES E. VAN HORN, Primary Examiner

R. E. MARTIN, Assistant Examiner

U.S. Cl. X.R.

UNITED STATES PATENT OFFICE  
CERTIFICATE OF CORRECTION

Patent No. 3,672,930 Dated June 27, 1972  
Inventor(s) William Trachtenberg

It is certified that error appears in the above-identified patent  
and that said Letters Patent are hereby corrected as shown below:

Column 18, line 4, cancel "liquid", first occurrence.

Signed and sealed this 27th day of February 1973.

(SEAL)  
Attest:

EDWARD M. FLETCHER, JR.  
Attesting Officer

ROBERT GOTTSCHALK  
Commissioner of Patents